

# UNITED STATES PATENT OFFICE.

JOSEPH NUSBAUM, OF PHILADELPHIA, PENNSYLVANIA, ASSIGNOR TO P. E. SHARPLESS COMPANY, OF PHILADELPHIA, PENNSYLVANIA, A CORPORATION OF PENNSYLVANIA.

## METHOD OF PACKAGING AND SEALING PERISHABLE ARTICLES AND THE PRODUCT THEREOF.

1,399,270.

Specification of Letters Patent.

Patented Dec. 6, 1921.

No Drawing.

Application filed June 7, 1920. Serial No. 387,224.

To all whom it may concern:

Be it known that I, JOSEPH NUSBAUM, citizen of the United States, and resident of Germantown, Philadelphia, State of Pennsylvania, have invented certain new and useful Improvements in Methods of Packaging and Sealing Perishable Articles and the Product thereof, of which the following is a full, clear, and exact description, reference 10 being had to the accompanying drawings, forming a part of this specification.

My invention relates to packaging and sealing, to preserve from moisture and natural deterioration, small perishable articles, especially rolls of soft or uncured cheese. This article of food has heretofore and now been commercially packaged and sold in small rolls, which are inclosed in metal foil, such as either tin foil or aluminum foil, not 15 only for sanitary purposes but to enable them to be more readily handled in commerce and to protect them from exposure to the air and its decomposing effects. Such method of packaging answers all these purposes satisfactorily, except the last named; and the single ultimate object of my invention is to seal the package in order to extend the life of the contents in sweet and edible condition.

To this end my invention consists broadly 20 stated, in a novel method and means of producing a sealing effect on the foil-inclosed roll of cheese or other perishable edible, and in the sealed package as the resultant product thereof.

The attainment of the ultimate object 25 stated, involves primarily the employment with melted paraffin of a combining element in a melted admixture with the paraffin, to cause it, when applied as hereinafter 30 stated to effect a coating of the metal foil with a fixedly adhering thin film of paraffin, and secondarily of a novel method of applying the melted admixture to the package, the employment of the combining ingredient 35 and the method of applying the mixture resulting in a coating of paraffin on the entire package, that will not loosen or peel therefrom under flexure. I apply such means and that method as a basis for the present 40 invention of a sealed package, and which I will now describe.

A small sheet of tin foil or aluminum foil, of a size sufficient to pass around the cheese

roll in the direction of its length and fully overlap at the edges and also extend beyond each end of the roll sufficient to be folded on itself to inclose the cheese roll, is employed to form thereby a covering over the entire roll. This is now the usual and common practice. It is so packaged for sanitary reasons and to provide a more readily handled product for commercial reasons. With such cheese, as the product packaged, there is no adequate exclusion of air and moisture, and obviously a constant liability to deteriorate 55 in quality, if not in character, in a few days.

I have improved this character of packaging by a subsequent paraffin sealing, which when applied by the means and in the manner hereinafter described, will be effective to 60 exclude air and moisture therefrom to such extent as to very materially prolong the "keeping" quality of the contents, besides 65 excluding all foreign matter, and hence make the contents more sanitary.

In carrying out my process to produce such a sealed package, by means of a coating of paraffin as a sealing medium, it is desirable not only to make this coating as a very thin and transparent film so that the descriptive 70 printing or label usually printed directly on the surface of the foil may be clearly seen, but essential to cause such a substantial adherence of the paraffin film to the foil that 75 it will practically unite with or firmly adhere to the surface thereof, sufficiently, at least, to prevent loosening or peeling therefrom under flexure due to ordinary handling 80 of the sealed package.

I am aware that efforts have been made 85 heretofore, by means of preliminarily-applied heat to tin foil, and simultaneously-applied pressure to both elements, to so attach a thin coating of paraffin to one or both sides of the foil, but my process differs radically therefrom, and the products of each are not comparable in the quality of adherence 90 above referred to; my product responding satisfactorily to flexure without loosening or peeling off, and is productive of extreme 95 thinness of the deposited coating, which is substantially transparent.

I have found from repeated experiments 100 that pure beeswax will when a very small percentage of resin is added, both admixed 105 with the melted paraffin, cause the paraffin

to effectually attach itself to the surface of the foil so as practically to become a fixed part of its surface; and I have further found that dipping the foil into a hot body 5 of the said composition, rather than pouring or otherwise similarly applying melted paraffin to a fixed body of the foil, whether the latter be hot or cold, effects not only a thinner and more transparent deposit there- 10 on of the paraffin coating but a more even distribution of it; and that dipping takes up less unnecessary quantity of the paraffin, which, if promptly followed by a slight vibration of the coated foil on a suitable holder 15 removes substantially all surplus, leaving an exceedingly thin and transparent coating, fixedly attached to the surface of the foil and capable of flexure without disturbing the adherence of the coating under ordinary 20 commercial usage.

In the practice of my process, I use commercial tin-foil, or commercial aluminum foil, of a suitable thickness for the purpose to which it is to be ultimately used; and 25 commercial paraffin of a grade which is white in color, is known as a purified product of the distillation of crude petroleum and a by-product in the manufacture of gasolene, and melts at a temperature varying 30 from about 122 to 127° F.; pure natural beeswax, preferably excluding any adulterated commercial beeswax, which is a light lemon in color and has a melting point of about 65° C. or very nearly the same as pure 35 paraffin; and commercial resin, which, if pure and unadulterated softens at 70° C. and melts at 100° C.

Applying the process practically I melt in a suitable vessel, the said ingredients, in the 40 proportion of 85 parts by weight, of paraffin, and 15 parts of beeswax and resin, the latter not exceeding 5 parts.

As commercial resin usually contains some non-soluble material or some part thereof 45 which is not readily soluble at the melting temperature to which the other elements are subjected, I recommend that it be suspended in the melting pot in a thin textile bag which will allow the soluble portion to ooze 50 through the bag while retaining the non-soluble remainder, hence maintaining the clarity and fluidity of the paraffin and wax solution. These being melted and admixed, the previously prepared package is dipped 55 in the vessel, by any suitable means, a single dipping being sufficient to attach thereto a suitable coating, and then withdrawn and immediately laid in a moving bath of cold water, on a wire frame or other suitable 60 holder, prior to which, if desired, the frame

may be slightly vibrated to shake off surplus coating and reduce the thickness of the coating to that which will adhere before it sets. To produce the best results I have found that the temperature of the solution, after 65 melting takes place, should be raised to 212° F. or 100 C. or even slightly above this, to increase its fluidity, at the time of dipping the package, the effect of which is to deposit on the package a relatively thinner and hot 70 coating more easily deprived by a slight vibration recommended of any surplus coating taken up, and avoiding any "setting" action prior to the application of the water bath. 75

Having thus described my invention, I claim:

1. The process of packaging and sealing perishable articles, which consists in forming a closed package by completely inclosing 80 the article in a sheet of metal foil, such as tin foil or aluminum foil, preparing a melted paraffin composition containing beeswax and resin, raising the temperature thereof to effect complete fluidity, and dipping the 85 package therein to effect a sealing coating thereon throughout the entire exterior surface of the package.

2. The process of packaging and sealing perishable articles, which consists in forming a closed package by completely inclosing 90 the article in a sheet of metal foil, depositing on the exterior of the package a melted paraffin composition containing beeswax and resin, subjected to a temperature sufficient to 95 effect complete fluidity, and setting the coating by a water bath.

3. The process of packaging and sealing perishable articles, which consists in forming a closed package by completely inclosing 100 the article in a sheet of metal foil, depositing thereon a coating of a fluid composition of paraffin, resin and beeswax at a high temperature, vibrating the coated package to remove surplus coating, and setting the coating by a water bath. 105

4. The new product described which is a sealed package comprising an inclosing wrapper of metal foil such as tin or aluminum foil, having fixedly adhering to the 110 entire exterior of the inclosing foil wrapper a sealing coating consisting of a composition of paraffin, resin and beeswax.

In testimony whereof I have hereunto affixed my signature this third day of June, 115 A. D. 1920.

JOSEPH NUSBAUM.

Witnesses:

I. M. TUNIS,  
ALEXANDER PARK.